

# United States Patent [19]

Fang et al.

[11] 4,137,685

[45] Feb. 6, 1979

[54] **SULFUR-COATED BAMBOO REINFORCEMENT MEMBER FOR CONCRETE ARTICLES**

[76] Inventors: **Hsai-Yang Fang**, 1847 Markham Dr., Bethlehem, Pa. 18017;  
**Harshavardhan C. Mehta**, 37-A Southern Ave., Calcutta, 700029, India

[21] Appl. No.: 784,686

[22] Filed: Apr. 5, 1977

[51] Int. Cl.<sup>2</sup> ..... E04C 3/36

[52] U.S. Cl. ..... 52/727; 52/733; 52/737; 427/204; 427/291; 427/440; 428/17

[58] Field of Search ..... 52/722, 577, 576, 727, 52/737, 659, 733; 242/7.22; 427/291, 204, 440; 428/17

[56] **References Cited**

**U.S. PATENT DOCUMENTS**

825,870 7/1906 Schirra ..... 427/204 X  
1,006,173 10/1911 Aine ..... 242/7.22

1,018,624 2/1912 Kolossvary et al. ..... 427/291  
1,617,447 2/1927 Johnston ..... 52/722

## OTHER PUBLICATIONS

Perry; John H. (ed.), Chemical Engineers' Handbook, 3rd ed., 1949, McGraw-Hill Book Co., New York City, pp. 1241-1242.

Primary Examiner—Ronald H. Smith  
Assistant Examiner—Evan K. Lawrence

[57] **ABSTRACT**

A reinforcement member for concrete bodies includes a bamboo rod having a roughened surface consisting of the bamboo cortex, and a substantially continuous coating of crystallized sulfur adhering to the roughened surface to prevent moisture absorption and swelling of the bamboo rod. The rod may have a helical wrapping of wire to further prevent swelling. The manufacture of the member includes roughening the rod by removing the bamboo article to expose the cortex, and dipping the rod in a bath of molten sulfur coating.

**5 Claims, No Drawings**

## SULFUR-COATED BAMBOO REINFORCEMENT MEMBER FOR CONCRETE ARTICLES

### BACKGROUND OF THE INVENTION

Bamboo is one of the fast growing perennial grasses. Individual rods of bamboo, referred to as culm, are divided into sections by joints or knobs referred to as nodes. In many parts of the world, bamboo is utilized as a low-cost construction material. When individual rods are utilized as a reinforcement member for concrete or cementitious bodies, the bamboo absorbs moisture from the fresh concrete. As bamboo absorbs the water, swelling occurs, and the volume of the bamboo increases. If the swelling pressure is large enough, the bamboo pushes the wet concrete aside. At the end of the curing period, (approximately 21 days), the concrete becomes hard, the bamboo has lost its water and shrinks, leaving voids between the bamboo rod surface and the concrete.

Such voids can trap air, moisture, and other foreign materials which will accelerate decay of the bamboo rod, causing cracks in the structure. Also, voids lead to a loss of bond, or adherence, between the bamboo and surrounding concrete.

It is well known to coat the bamboo rods with various materials, such as paint, tar, cement, and asphalt emulsion, in order to reduce the water absorption potential of bamboo. Unfortunately such techniques are either too expensive or ineffective due to difficulty of application.

Therefore, there is a need for a treated bamboo which can resist swelling due to absorption of moisture, and thereby prevent loss of bond with surrounding concrete in a reinforced concrete body.

### SUMMARY OF THE INVENTION

The present invention provides a moisture resistant, non-swelling bamboo reinforcement member for concrete comprising a roughened bamboo surface, the bamboo cortex, and a substantially continuous coating of crystallized sulfur contacting and adhering to the cortex to prevent moisture absorption and swelling of the bamboo rod. The rod may have a helical wrapping of wire to further prevent swelling. In an alternate embodiment, the sulfur coating has particles of sand embedded therein.

### DESCRIPTION OF PREFERRED EMBODIMENTS

In the preferred embodiment, the swelling resistant sulfur-coated bamboo is produced according to the following procedure:

Bamboo rods are first dried to remove moisture. Drying can be in a conventional drying oven or by air drying. For air drying, a period of up to two months is recommended.

The smooth outer skin of the bamboo is roughened. By roughened, we mean that the waxy cuticle of the bamboo epidermis is removed, to cause proper adherence of sulfur and bamboo. We have discovered that crystallized sulfur will not adhere to the bamboo properly after hot-dipping unless the smooth outer bamboo skin is removed.

We believe that proper adherence of sulfur is a result of the molten sulfur contacting the cortex below the epidermis and penetrating and adhering to the fibers known as sclerenchyma fibers, which fibers, as is well

known, surround the irregularly spaced vascular bundles of the bamboo culm.

We prefer to roughen the surface, or remove the bamboo cuticle, by conventional sand blasting, although other mechanical means, such as stripping with cutters or grinders can be used, as well as chemical means such as acid stripping.

Wire is wrapped in a helical fashion around the rod to prevent swelling. However other materials, such as a rope, will work.

The bamboo rod is soaked, or hot dipped, in molten sulfur for about one hour. The time is not critical. The sulfur temperature should be maintained between 238° F. and 300° F., a temperature at which molten sulfur has low viscosity, enhancing sulfur penetration into the bamboo fibers. If the temperature is too high, the bamboo may burn, and if the temperature is too low, the sulfur is too viscous. After the hot dipping period, the bamboo is air dried to form a substantially continuous, 20 impervious coating of crystallized sulfur on the bamboo.

It is important that the sulfur coating be continuous, that is, have no gaps, leaving bare spots of exposed bamboo. In other words the sulfur coating must not 25 have any pinhole openings, which pinholes could permit moisture penetration.

Multiple coatings can be used, but the bond between bamboo and surrounding concrete is not significantly improved, although more sulfur improved the bending stress of the bamboo.

We prefer to apply sulfur in an amount between 5% and 15% by weight of the starting bamboo rod, or equivalently, a thickness of coating between 1 to 6 mm.

We prefer to use commercial grade flour sulfur, 35 99.9% purity, having, as a solid, a specific gravity of 2.08. Such sulfur, as is well known, has mainly two allotropes, the alpha (rhombic) and beta (monoclinic) phases. The rhombic phase is the stable form at temperatures up to 203.9° F., and therefore, the crystallized, 40 continuous, elemental sulfur coating on the bamboo rods is in the rhombic phase.

We believe that common impurities in the sulfur can be present without deleterious effects. Such impurities can include acid, ash, and other carbonaceous compounds in the range commonly found in sulfur.

As an alternate embodiment, sand can be applied to the sulfur before the sulfur has completely crystallized, or dried. Sand increases the bond between bamboo and concrete.

To illustrate the effectiveness of a crystallized-sulfur-coated bamboo rod in concrete, the following example is described.

### EXAMPLE I

Bamboo specimens were air dried for two months. The smooth bamboo skin was removed by sand blasting, and 28 gage wire helically wrapped around some of the rods. Specimens were soaked for about one hour in molten sulfur at a temperature around 280° F. to 300° F. 55 Sand was applied to the sulfur coating before it completely dried.

Each bamboo rod was inserted into a cylindrical form containing concrete of the following analysis by volume: one part cement, ASTM standard type A, four parts aggregate, two parts sand, and a water to cement ratio of 0.4 to 0.55.

After a curing period of 21 days, the bond stress was measured by determining the force required to pull the

bamboo out of the concrete, or to break the rod if it did not come out.

Table I shows the results for a bamboo rod having no nodes immersed in the concrete.

Table I

| Type Sample          | Pull Force - lbs. |
|----------------------|-------------------|
| Untreated Bamboo     | Pulled out        |
| Sulfur-Coated Bamboo | 2315              |
| Sulfur-Coated Bamboo |                   |
| Wrapped with Wire    | 2380              |

Table I illustrates a significant increase in bond stress resulting from the treated bamboo of this invention.

Of course, for specimens having nodes within the concrete, the pull force may vary due to the added resistance to slipping presented by the nodes alone.

Examination of similarly treated specimens was done by sectioning the concrete parallel to the length of bamboo to determine whether or not voids developed between the bamboo surface and surrounding concrete. In all cases, untreated bamboo exhibited voids and decreased adherence of concrete due to the swelling and subsequent shrinkage of bamboo, as hereinbefore described.

All bamboo treated according to the invention had substantially no void formation between the bamboo surface and surrounding concrete. The concrete substantially completely contacted and adhered to the sulfur-coated surface of the bamboo.

We believe it would be equivalent to split individual bamboo rods lengthwise and utilize them as reinforcement members for concrete bodies pursuant to the teaching of the invention disclosed herein.

We also believe it within the scope of this invention to sulfur coat the internal surface of the bamboo culm,

in accordance with the teachings herein, to produce a hollow conduit suitable for conducting water without swelling.

We claim:

- 5 1. A reinforcement member for concrete bodies comprising:
  - (a) a bamboo rod having a roughened surface said roughened surface being a bamboo cortex without a waxy cuticle of epidermis; and
  - (b) a substantially continuous coating of crystallized sulfur contacting and adhering to said cortex of said bamboo rod, to prevent moisture absorption and swelling of said bamboo rod.
- 10 2. The reinforcement member of claim 1 further including wire wrapped around said rod and embedded in said sulfur coating.
- 15 3. The reinforcement member of claim 2 further including sand particles embedded in said sulfur coating.
- 20 4. The reinforcement member of claim 3 in which the sulfur coating is present in a thickness between 1 mm to 6 mm.
- 25 5. A reinforced concrete article comprising:
  - (a) a concrete matrix;
  - (b) a crystallized-sulfur coated bamboo rod embedded in said concrete matrix and contacting said concrete matrix substantially free of voids between said sulfur coating and concrete matrix;
  - (c) said bamboo rod having a bamboo cortex without a waxy cuticle of epidermis; and
  - (d) said sulfur coating contacting and adhering to said bamboo cortex in a substantially continuous fashion to prevent moisture absorption and swelling of said bamboo rod.

\* \* \* \* \*